# EUROPEAN PATENT SPECIFICATION

(11) **EP 0 236 478 B1**
(45) Date of publication and mention of the grant of the patent: **15.01.1997**
(21) Application number: 86906054.1
(22) Date of filing: 09.09.1986
(51) Int. Cl.: B32B 5/16, B32B 5/20

(54) **DECORATIVE INLAID TYPES OF SHEET MATERIALS**
BLATTMATERIALIEN MIT EINLEGEDEKOR
TYPES DE MATERIAUX EN FEUILLE A INCRUSTATIONS DECORATIVES

(30) Priority: 09.09.1985 US 773984
(43) Date of publication of application: 16.09.1987
(73) Proprietor: TARKETT, INC., Parsippany, NJ 07504 (US)
(72) Inventor: LUSSI, Edward, Franz, Bethlehem, PA 18018 (US); SMITH, Thomas, George, Easton, PA 18042 (US)
(74) Representative: Paget, Hugh Charles Edward
(86) International application number: US8601849
(87) International publication number: WO8701334

(56) References cited:
- EP-A- 0 085 784
- FR-A- 2 572 022
- US-A- 3 239 364
- US-A- 3 856 900
- US-A- 4 196 243
- US-A- 4 212 691
- US-A- 4 239 797
- US-A- 4 440 826
- US-A- 4 450 194

## Description

### Field of the Invention

The present invention relates to decorative inlaid sheet materials and the like. More particularly the invention is concerned with the use of polyvinyl chloride (hereinafter "PVC") polymerization agglomerates as decorative particles and their application on floor and wall covering substrates to produce realistic inlaid patterns, utilizing heretofore unobtainable design strategies and exhibiting superior properties.

The particles can be spherical and, when such is the case, are hereinafter sometimes referred to as "pearls". These pearls can be random-sifted on the substrate or applied in geometrical patterns. Also disclosed is the use of mixes or blends containing transparent or partly transparent pearls allowing visible underprinting as a further strategy for unique design variations.

### Background of the Invention

Sheet materials, in particular sheet vinyl flooring products, made with chips or particulate material, are commonly referred to as inlaids. These products and processes for their manufacture are well known in the floorcovering business and originate back to the early linoleum times where through patterned floorcoverings, based on linseed oil, cork dust and resins were developed by the industry. The process was later modified for vinyl.

Vinyl inlaid floorcovering consists of coarse colored particles, such as chips or dry blends, which are "laid on" a substrate and then sintered by heat, or "laid in" a transparent liquid or solid matrix and fused by heat. The chips are produced from pre-gelled or fused spread, calendered or extruded compounds cut into geometrically regular profiles or ground into randomly shaped particles.

The dry blends are made by mixing fine PVC powder with plasticizer, filler and color pigments and heating above the PVC compound's softening temperature. The small original particles "grow" and form a loose, porous, coarse, fluffy mass.

Currently, to produce realistic inlaid patterns for sheet vinyl, conventional manufacturing procedures distribute the coarse particles on the substrate in different steps with the help of area-complementary stencils, followed by topcoating with a clear wearlayer. This method is complicated and can only be used to produce large geometric patterns.

The inlaid floorcoverings are normally characterized as those which maintain their decorative appearance as the surface is worn or abraded away. This characteristic makes such products particularly suitable for use in commercial areas where significant wear is encountered.

Modern inlaids generally fall into two classifications: resilients and non-resilients. Resilients include a substantially continuous layer of foam and are usually made by incorporating solid particulate material into a plastisol coating, followed by gelling and fusing. Non-resilients do not contain a foam layer and usually are made by sintering and/or calendering, or otherwise compacting, particulate material.

The non-resilient products commercially offered are those containing large (about 3 mm, i.e 1/8 inch) square chips in a clear matrix and those containing small (about 0.1 mm, i.e 0.004 inch) dry blend resin particles made by sintering and/or compacting normal dry blend resins. It is believed that the reason no products containing chips, granules, or particles of an intermediate particle size, for example ranging from 0.1 to 1.0 mm (0.004 inch to 0.040 inch), are offered results from limitations inherent in current inlaid manufacturing technology, discussed more fully hereinafter.

While construction of inlaid products by compaction from discreet chips or particles (normally of different colors) offers distinct styling opportunities, a significant premium is paid in terms of expensive, cumbersome equipment. Furthermore, the nature of the process restricts the range of designs available. For example, in order to effect specific registered pattern definition, it is necessary to deposit chips of different colors in preselected areas on the sheet. This is difficult mechanically, and results in a slow cumbersome process which does not produce finely defined designs.

Some of the inherent difficulties in current production techniques for non-resilient inlaids have been minimized by use of increasingly sophisticated materials and design techniques, such as using fine particle size, dry blend resins, printing over the surface of the resulting inlaid product, optionally, embossing, with and without application of a wearlayer. Unfortunately, whereas the use of the finer particle size preserves the specific characteristic of an inlaid product, ie. the pattern does not change as the product wears through, overprinting the product, whether or not a wear layer is applied, essentially negates this characteristic because wearing through the print layer essentially destroys the pattern. This eliminates the product from commercial, high-use environments and limits its utility principally to styling effect in residential and related applications.

Resilient inlaids are usually made by embedding ground plastic particulate material in a plastisol coating. US-A-4,212,691 exemplifies such product and methods for their manufacture. As taught in this patent, the thickness of the particles of the decorative chips or flakes is stated to be from about 0.075mm (3 mils) to about 0.62mm (25 mils): see for example column 7, lines 62-64. However, it is the length of the particle, ie. its largest dimension, rather than thickness that is observed when viewing the pattern. That dimension is stated to be from about 1.2mm to 12mm (50 to 500 mils) at column 8, lines 17-18. It is to be noted that the products disclosed all contain embedded chips or flakes ground from plastic sheet stock, even when chips or flakes from other stock materials are added (eg. see column 8, lines 4 et seq). These chips or flakes characteristically have a high aspect ratio (ie. length/thickness).

Other disclosures of products with applied chips or flakes are US-A-3,239,364 which discloses pressing solid particles into a printed base coat and US-A-4,440,826 which discloses a product in which transparent chips are pressed into an opaque layer until they create windows exposing a printed layer below. US-A-4,196,243 discloses particles incorporated into a wearlayer so as to provide a non-slip wearlayer over a pigmented rather than printed base.

US-A-4,450,194 discloses decorative coverings for floors and walls in which resin particles are used to provide differentials in gloss and texture. This document discloses an arrangement in which a vinyl plastisol ink is applied to selected areas registering with a printed image applied to a substrate. Resin particles are applied and adhere to the plastisol ink in the selected areas only. A top layer of PVC plastisol over the entire product provides a smooth surface outside the selected areas but leaves the particles projecting above the surface in the selected areas, thus giving selected areas of greater texture and lower gloss. In between these areas, the surface is smooth.

Thus, existing inlaid technology, although capable of producing commercially satisfactory inlaid products, has limitations and deficiencies. State of the art inlaid technology for "chip" products first grinds the chips from plastic sheets. This predefines the particle shape and is expensive. Furthermore, spherical particle shapes cannot be made by the grinding techniques currently in use for inlaids.

Additionally, products formed by compacting or sintering dry blends have always shown limited particle distinction due to process limitations and available particle sizes. The particles tend to lose their identity due to agglomeration or lumping caused by sintering process.

### Purposes and Objects of the Invention

It is, therefore, a principal purpose and object of this invention to provide heretofore unobtainable real through patterned inlaids, offering unique design advantages and flexibility, as well as superior properties. For example, wear resistance is significantly increased in comparison with leading commercially available inlaids. It is also a primary purpose and object of this invention to provide a novel process for producing such inlaids which is believed to be simpler and significantly less complicated than state-of-the-art inlaid production technology. Another purpose and object is to provide a process that in the main utilizes today's plastisol equipment and technology. Other principal purpose and objects of this invention will be apparent from the following discussion.

### Summary of the Invention

The foregoing and other purposes and objects of this invention are accomplished by providing a decorative, inlaid floor or wall covering product which incorporates as the essential elements thereof (i) resinous particles having an aspect ratio significantly lower than those currently employed in inlaids commercially offered in the United States, (ii) an adhesive matrix in which said particles are embedded, and (iii) a substrate which supports these over a print layer which is visible through the adhesive matrix layer.

Thus, the invention provides a decorative, inlaid floor or wall covering in the two forms as claimed in the claims

Preferably the particles have a size within a range from 0.1 to 1.0mm (0.004 to 0.04 inch). Preferably also the particles employed in this invention have as aspect ratio of no greater than 1.5:1. Particles having an aspect ratio of about 1:1 and, in particular, particles which are also spheroidal, are especially preferred because of the excellent results achieved therewith, as discussed more fully hereinafter. The use of particles which are essentially as thick as they are flat, ie. having a low aspect ratio, provides a product that will not lose its pattern due to wear in use, thus preserving the unique property which characterizes true inlaids.

The use of printed patterns which are visible beneath the adhesive matrix containing the particles broadens the options available to the pattern designer and constitutes another embodiment of this invention. Exemplary is a decorative, inlaid floor or wall covering which comprises:
a) a substrate,
b) a printed layer, generally comprising a printable substrate coating or sealant, onto which is printed a pattern in an ink suitable for floor or wall covering applications, applied over and in contact with said substrate, and
c) an adhesive matrix, overlaying said printed layer, and in contact therewith, in which are embedded the resinous particles, said matrix being sufficiently transparent or transluscent to permit the underprint to show through.
Such product provides options for a wide variety of design strategies heretofore unobtainable with state-of-the-art sheet vinyl technology and constitutes a preferred embodiment of this invention.

The inlaid products of this invention offer unique design advantages. Further, cost advantages can also be realized by utilizing raw materials which are believed to be unique to inlaid manufacture. For example, certain of the novel products of the invention incorporate an adhesive matrix consisting essentially of a plastisol layer containing a high loading of transparent and/or transluscent and colored, spheroidal resinous particles, which, preferably, range in size from 0.1 to 1.0 mm (0.004 inches to 0.040 inches). When this matrix is applied over a printed pattern, a unique visual effect is produced.

Such particles can be made in uniform controlled sizes by employing technology described in United States Patent 3,856,900. Alternatively, special large particle size dry blend resinous particles, either screened to the desired size ranges of this invention from oversized material obtained from normal production variations, or specially made particles in the desired size range, can be utilized.

Another, and preferred, embodiment of this invention is a decorative, inlaid floor covering which comprises:
a) a non-asbestos felt sheet substrate,
b) a gelled, printable, plastisol coating over said substrate,
c) one or more solvent based PVC-polyvinyl acetate copolymer inks applied to the surface of the plastisol layer,
d) a gelled adhesive matrix, overlaying said plastisol/print layer, and in contact therewith, containing an effective amount of a homopolymer or a copolymer of vinyl chloride, in which are embedded discreet spherical and essentially spherical, gelled and resinous particles, at least some of which permit the underprint to show through, and wherein said particles are coarse PVC homopolymer or copolymer polymerization agglomerates, sized to between 0.1-1.5 mm (0.004-0.060 inches) preferably less than 1.0 mm (0.040 inches) and, optionally,
e) a fused, transparent, plastisol wearlayer as a top coat.

### General Description of the Invention

The product is comprised of a base supporting material, which, optionally, may be precoated with a plastisol to enhance printability, a print layer offering decoration, and an adhesive matrix containing transparent and pigmented resin particles, which are preferably spherical or spheroidal. In one embodiment the resulting product has an additional coating on its top surface to enhance surface properties, such as gloss and the like, and insure there is no residual porosity resulting from the process of embedding the particulates in the adhesive matrix.

The incorporation of particulate materials of such size and shape, and at the loadings herein described provides the retention of pattern as the product wears through characteristic of inlaid products. The incorporation of transparent particles allowing the underprint to show through, provides an additional dimension in design capability. The combination of a transparent or transluscent adhesive matrix loaded with transparent or transluscent and/or pigmented or colored particulate material and the use of rotogravure or other forms of print offering fine registered detail and definition, provide a product which is believed to be unique and a significant advance in the art.

One of the advantages of this invention is that it employs ingredients and processing technology well known to those skilled in the art. Also, by employing a fluid plastisol as the matrix material binding the particles together, the product can be manufactured without the need for the high pressures or temperatures characteristic of the calendering or agglomeration steps of the prior art processes. This processing characteristic also distinguishes the subject process from those of the prior art which employ only dry blend resins, which are agglomerated through heat sintering.

### Substrate

The substrate is a relatively flat fibrous or non-fibrous backing sheet material, such as a fibrous, felted or matted, relatively flat sheet of overlapping, intersecting fibers, usually of non-asbestos origin. The substrate can, if desired, be asbestos or non-asbestos felts or papers, woven or non-woven; knitted or otherwise fabricated textile material or fabrics comprised of cellulose, glass, natural or synthetic organic fibers, or natural or synthetic inorganic fibers, or supported or non-supported webs or sheets made therefrom or filled or unfilled thermoplastic or thermoset polymeric materials. These and other substrate or base materials are well known in the art and need not be further detailed here.

### Substrate Coating

The substrate or base material, optionally, can be coated to improve the print quality of the substrate. Such coatings can be plastisols, organosols, lacquers, filled or unfilled latex coatings, or other coatings conventionally employed as preprint sealants in the manufacture of floor or wall covering products.

As used herein, the term "plastisol" is intended to cover a relatively high molecular weight polyvinyl chloride resin dispersed in one or more plasticizers. The plastisol upon heating or curing forms a tough plasticized solid. For purposes of the present invention plastisol compositions are intended to include organosols, which are similar dispersed polyvinyl chloride resin materials that, in addition, contain one or more volatile liquids that are driven off upon heating.

Those skilled in the art will appreciate that, in addition to the basic resin constituents, other commonly employed constituents can be present in the plastisol compositions in minor proportions. Such other constituents commonly include heat and light stabilizers, viscosity depressants, and/or pigments or dyes, the latter in order to contribute color to the polyvinyl chloride resin.

Typically the substrate coating employed in the products of this invention is a resinous polymer composition, preferably, a polyvinyl chloride plastisol which is substantially uniformly applied to the substrate surface, for example by means of a conventional reverse roll coater or wire wound bar, eg. a Meyer Rod Coater, wherein the grooves provided by the wires assist in metering the flow of the plastisol. The particular means for applying the substrate coating to the surface of the substrate does not relate to the essence of the invention and any suitable coating means can be employed. Exemplary of other coating means are knife-over roll coater, rotary screen, direct roll coater and the like.

The thickness of the resinous polymer composition or plastisol, as it is applied to the surface of the substrate, is substantially uniform, and is preferably in the range of 0.075 mm to 0.75 mm (3 mils to 30 mils). The substrate can be thinner or thicker as may be required by the particular product application.

Although the preferred and typical substrate coating is a polyvinyl chloride homopolymer resin, other vinyl chloride resins can be employed. Exemplary are a vinyl chloride-vinyl acetate copolymer, a vinyl chloridevinylidene chloride copolymer, and copolymers of vinyl chloride with other vinyl esters, such as, vinyl butyrate, vinyl propionate, and alkyl substituted vinyl esters, wherein the alkyl moiety preferably is lower alkyl containing between about 1-4 carbons. Other suitable synthetic resins such as polystyrene, substituted polystyrene, preferably wherein the substituents are selected from the group consisting of alkyl (C₁-C₁₀, preferably C₁-C₄), aryl (preferably, C₆-C₁₄), polyolefins such as polyethylene and polypropylene, acrylates and methacrylates, polyamides, polyesters, and any other natural or synthetic resin capable of being applied to the substrate or base coatings of this invention to provide a smooth and uniform surface and/or to improve the print quality of the substrate or base coating surface, are also applicable; provided such resin is otherwise compatible with the overall product composition and, therefore, within the principles of this invention. Thus, it is not essential that a plastisol always be used. Organosols and aqueous latices (aquasols and hydrosols) are also of use, employing as the dispersing or suspending media, organic solvents and water, respectively, rather than plasticizers, as in the case of a plastisol.

Where the preferred plastisol is employed, typical of the plasticizers which can be used are dibutyl sebacate, butyl benzyl sebacate, dibenzyl sebacate, dioctyl adipate, didecyl adipate, dibutyl phthalate, dioctyl phthalate, dibutoxy ethyl phthalate, butyl benzyl phthalate, dibenzyl phthalate, di(2-ethylhexyl) phthalate, alkyl or aryl modified phthalate' esters, alkyl, aryl, or alkylaryl hydrocarbons, tricresyl phosphate, octyl diphenyl phosphate, dipropylene glycol dibenzoate, dibasic acid glycol esters, and the like. Other constituents of the resinous substrate coating can include a blowing or foaming agent such as azodicarbonamide (if a blowing or foaming procedure is desired), conventional stabilizers/ accelerators, initiators, catalysts, etc., such as zinc oleate, dibasic lead phosphite, etc., conventional heat or light stabilizers, such as metallic soaps, etc., UV absorbers, colorants, dyes or pigments, notably, titanium oxide, solvents and diluents, such as methyl ethyl ketone, methyl isobutyl ketone, dodecyl benzene, etc., fillers, such as clay, limestone, etc, viscosity modifiers, antioxidants, bacteriostats and bacteriocides, and the like.

### Print Layer

Suitable inks include those normally used in the manufacture of floor covering, preferably resilient floor covering. These include plastisol, solvent based systems and water based systems. Such systems can include a chemical suppressant in those cases where the substrate to which the ink is to be applied is a foamable plastisol or organosol. Such suppressants are well known in the art (eg. see US-A-3,293,094).

Printing onto the substrate can be effected by rotogravure, flexigraphic, screen printing, or other printing techniques conventionally employed in making floor or wall covering products.

### Adhesive Layer

The adhesive layer is normally a plastisol or organosol additionally containing a plasticizer system, associated diluents, viscosity control aids and stabilizers. Those discussed above are exemplary. When underprinting is present, the adhesive would not normally contain colors or pigments which would render the adhesive layer opaque.

Although other homopolymers and copolymers of vinyl chloride, (ie. vinyl resins other than a plastisol or organosol) such as those discussed above, can also be employed, as a practical matter, current economics dictate the use of polyvinyl chloride plastisols of the type set forth in the examples hereinafter.

### Resinous Particles

The resinous particles of this invention can be of various sizes and geometric shapes, spherical and essentially spherical, (sometimes referred to herein as "spheroidal") being especially preferred as having the low aspect ratios discussed herein required to obtain the desirable design effects this invention is capable of providing. Each transluscent or opaque particle can contain its own individual colorant, dye or pigment. It may be preferred that in some embodiments of this invention at least some of the particles are sufficiently transparent or sufficiently transluscent, to permit the printing on the print layer to show through the particles concerned.

Employing discreet spheroidal particles is advantageous for enhanced visual effect of depth and improved wear characteristics. Illustrative of those spheroidal particles which are especially preferred are the particles and the methods for their manufacture taught in US-A-3,856,900. This procedure is particularly convenient for the production of relatively small plastisol beads or "pearls" having a particle size of generally about 0.75mm (0.030 inch) or smaller.

Particles can also be obtained by screening the oversized particles from normal suspension grade resin production or by making special particle sizes, for example, in accordance with US-A-3,856,900. Particles in this size range are particularly useful for achieving certain desirable design effects. Such procedures are also capable of making smaller particle sizes.
(eg. see US-A-3,345,235), but in the case of spheroidal particles, the procedure of US-A-3,856,900 is preferred.

Although spherical or essentially spherical particles are preferred, in general, the particles employed in this invention can have a wide variety of geometric shapes, provided that the aspect ratios of such particles fall within the ranges discussed herein. Exemplary of other geometric outlines are squares, triangles, circles, annuli, other polygons, etc, or irregular sizes and shapes, or a mixture of any or all of such shapes, including spheroidal.

It has been found that the size of the particles employed in carrying out this invention have a pronounced effect on the results obtained. Use of relatively small particles, eg. ranging from about 150 µm (100 mesh) to about 600 µm (30 mesh) are most advantageous in producing the desired design effects. Particles, especially spheroidal particles, averaging about 600 µm (by microscopic observation) are especially preferred.

The ratio of transparent to colored particles determines the visibility of the printed pattern underneath the resulting adhesive matrix. Generally, 50% or less, and preferably 0-30 %, transparent to colored particle loading is preferred. The amount actually used will, of course, depend upon the type of end-use application and design effect desired. Good results have even been achieved in the range of 0-10% transparent to colored particle loading.

### Wearlayer

The optional overcoat or wearlayer is preferably a plastisol of the same or similar type as that discussed above in connection with the resins employed in the substrate coat and the adhesive layer or matrix. The formulations generally include materials to enhance special specific properties, for example gloss, wear, stain resistance, and scuff resistance.

Other resins suitable for use as a top coating can be employed. Exemplary are wear resistant polyurethanes, such as those described in US-A-4,087,400.

Thus in another embodiment of this invention the decorative, inlaid floor or wall coverings comprise:
a) a flexible mat substrate,
b) a gelled, resinous print layer, applied over said substrate, the surface of which is printed with one or more inks suitable for use in the manufacture of floor or wall covering products, and
c) an adhesive matrix, overlaying said print layer, containing an effective amount of a homopolymer or a copolymer of vinyl chloride, and in which are embedded resinous particles, at least some of which permit the underprint to show through, and
d) an optional topcoating or wearlayer or wearlayers selected from the group consisting of a plastisol, a polyurethane resin or a suitable mixture of each.

The following examples are intended to demonstrate preferred embodiments of this invention without limiting the scope thereof. In the following examples all parts and percentages are by weight. PLIOVIC, IRGASTAB, SYNTRON, REVIKON, SYNPRON, TARKETT, ARMSTRONG, CONGOLEUM and FORBO are Registered Trade Marks.

### Example 1

### Floor Covering with Overall Pattern Suitable for Commercial Uses

A floor covering substrate sheet of conventional type non-asbestos felt (Tarkett Inc., Whitehall, Pa.), approximately 0.80 mm (32 mils) thick, was bar coated (wire wound bar) with approximately 0.075 mm (3 mils) of a layer of white printable plastisol, the composition of which was as follows:

| | Parts by Weight |
|---|---|
| PVC emulsion: relative viscosity 2.05 (Occidental FPC 605) | 70 |
| PVC extender: k value 60 (PLIOVIC M-50) | 30 |
| Di(2-ethylhexyl) phthalate | 30 |
| Butyl benzyl phthalate | 30 |
| Titanium dioxide | 5 |
| Crystalline calcium carbonate | 80 |
| Barium-zinc type stabilizer (IRGASTAB BZ 530) | 3 |

After gelling against a heated chromium drum at 149°C (300°F.), the resulting smooth surface is gravure printed on a flat print press using Series 125 inks from American Inks, Inc..

After drying in warm air at about 60°C (140°F.), an adhesive layer about 0.25 mm (10 mils) thick was applied by drawdown bar and an excess of premixed plastisol pearls (produced in Example 3 and having the composition set forth hereinafter), about half of which were transparent and the remainder colored, were evenly distributed on the surface of the wet, tacky adhesive layer from a vibrating pan (SYNTRON vibrator manufactured by FMC Corp.).The composition of the adhesive mix was:

| | Parts by Weight |
|---|---|
| PVC dispersion: (Occidental FPC 6458) | 70 |
| PVC extender: k value 60 (PLIOVIC M-50) | 30 |
| Butyl benzyl phthlate | 25 |
| Di-isononyl phthlate | 25 |
| Stabilizer, barium-zinc type (SYNPRON 1665) | 4 |

The composition of the pearl particles was:

| Parts by Weight | Colored | Transparent |
|---|---|---|
| Suspension grade PVC resin: k value 65 (PEVIKCON S658 GK) | 100 | 100 |
| Butyl benzyl phthalate | 40 | 40 |
| Stabilizer, barium-zinc type (SYNPRON 1665) | 4 | 4 |
| Titanium dioxide | 5 | -- |
| Color-pigment (Purchased blend of red iron oxide, yellow iron oxide and carbon black dispersed in di(2-ethyl-hexyl) phthalate) | 5 | -- |

The PEVIKON S658 GK resin had an aspect ratio of about 1 (the particles were round) and the particle size was found by microscopic observation to average about 600 µm (approximately 30 mesh). Screen analysis was as follows:

| Mesh | % Retained |
|---|---|
| 28 (589 µm) | 68.0 |
| 65 (208 µm) | 25.2 |
| 100 (147 µm) | 1.4 |
| Thru 100 mesh | 5.4 |

The excess pearls, which were not wetted by the adhesive coating and embedded therein were blown away by a gentle air stream. The resultant grainy matrix was then gelled by contacting the coated side against a heated chromium drum (177°C i.e 350°F.) and smoothed between a rubber pressure roller and the drum surface. The thickness of the matrix containing the adhesive coat (0.25 mm, i.e 10 mils) and the embedded pearls (approximately 0.5 mm, i.e 20 mils) was 0.75 mm, ie. 30 mils.

The surface of the matrix was then bar coated using a drawdown bar with a transparent plastisol wearlayer having the following composition:

| | Parts by Weight |
|---|---|
| Dispersion grade PVC, (Occidental FPC 6458) | 100 |
| Isobutyric acid and glycol ester of benzoic acid (Monsanto SANITIZER S-377 plasticizer) | 56 |
| Stabilizer, barium-zinc type (SYNPRON 1665) | 5 |
| Epoxidized soybean oil | 5 |
| Kerosene | 2 |
| Brookfield Viscosity: ∼1200 cps | |

The wearlayer was fused in a hot air oven at about 149°C (300°F.) for 3.5 minutes and then embossed between a cooled embossing roll and a rubber pressure roll. The resultant wearlayer has a thickness of about 0.38 mm (15 mils).

The wear characteristics of the decorative inlaid product thereby produced are set forth in the following Table I and compared with leading competitive products.

**TABLE I**

| TABER ABRASION Run on Taber Abrasion Model #505 using H-18 wheels | | | | | | | |
|---|---|---|---|---|---|---|---|
| PRODUCT | Initial Wt 4"X4" Smpl (g) | Caliper | | Wt. Loss % 1000 cycles (g) | Wear-out Point (cycles) | Product Thickness to Wear-out Point | |
| | | (mm) | (mils) | | | (mm) | (mils) |
| TARKETT | | | | | | | |
| Residential | 21.3014 | 2.34 | 92 | .0803 | 36,000 | 0.91 | 36 |
| Commercial | 22.3489 | 2.11 | 83 | .0919 | 60,500 | 1.14 | 45 |

| ARMSTRONG | | | | | | | |
|---|---|---|---|---|---|---|---|
| "Crowne Corlon" | 46.0910 | 1.90 | 75 | .2294 | 22,500 | 1.06 | 42 |
| "Designer Solarian" | 28.2392 | 2.24 | 88 | .2696 | 27,500 | 1.54 | 60.5 |
| "Solarian Supreme II" | 28.7303 | 2.34 | 92 | .3131 | 3,000 | 0.13 | 5 |

| CONGOLEUM | | | | | | | |
|---|---|---|---|---|---|---|---|
| "Innovation" | 17.2543 | 1.83 | 72 | .0905 | 8,000 | 0.25 | 10 |

| FORBO | | | | | | | |
|---|---|---|---|---|---|---|---|
| "Smaragd" | 18.1629 | 1.42 | 56 | .0416 | 24,000 | 0.69 | 27 |

### Example 2

### Residential Floorcovering with Registered Printed and Embossed Patterns (Chemically Embossed)

A floorcovering substrate sheet of conventional type non-asbestos felt (Tarkett Inc., Whitehall, Pa.) approximately 0.80 mm (32 mils) thick was coated with a foamable plastisol the composition of which was as follows:

| | Parts by Weight |
|---|---|
| PVC dispersion: k value 65 (Occidental FPC 605) | 70 |
| PVC extender resin: k value 60 (PLIOVIC M-50) | 30 |
| Di(2-ethylhexyl) phthlate | 28 |
| Butyl benzyl phthlate | 15 |
| Texanol isobutyrate (TXIB) | 15 |
| Titanium dioxide | 10 |
| Azodicarbonamide | 2.5 |
| Kerosene | 4 |
| Zinc oxide | 1.5 |
| Viscosity: 2500 cps | |

The coated substrate is then pregelled in a hot oven at 135°C (275°F.) for 2.5 minutes. The surface is then gravure printed on a flat bed press using inks having the same composition as those of Example 1 except that the inks used to cover the plate printing the valley areas of the pattern (ie. the grouts) contain additionally 140 parts benzotriazole, a chemical suppressant, to inhibit in these selected areas the expansion of the foamable plastisol.

After drying the print, an adhesive layer having the same composition as that of Example 1 was applied by a drawdown bar. Premixed colored and transparent pearls, in the same ratio as in Example 1, were evenly distributed, gelled and smoothed as described in Example 1. The thickness of the resulting matrix containing the pearls (0.38 mm, i.e. 15 mils) embedded in the adhesive (0.012 mm, i.e. 5 mils) was about 0.5 mm, i.e 20 mils. Approximately 0.25 mm, i.e. 10 mils of a transparent wearlayer having the same composition as that of Example 1 was applied with a drawdown bar. The resulting product was then fused and expanded (ie. foamed) in a hot air oven at 193°C (380°F.) for 3 minutes.

The floorcovering produced shows a relief structure (embossing) in register with the printed areas. The decorative inlaid product thereby produced has an overall thickness of about 2.08 mm (82 mils) and exhibited excellent wear and design characteristics.

### Example 3

The plastisol spherical "pearls" used in the foregoing examples were prepared using the following formulations:

| Parts by Weight | Colored | Transparent |
|---|---|---|
| Suspension grade PVC resin, coarse: k value 65 (PEVICON S658 GK) | 100 | 100 |
| Butyl benzyl phthalate | 40 | 40 |
| Barium-zinc stabilizer (SYNPRON 1665) | 4 | 4 |
| Titanium dioxide | 5 | -- |
| Color-pigment | 5 | -- |

In preparing the colored and transparent plastisol composition, the PVC resin (at 21°C, i.e 70°F.) was charged to a high intensity mixer running at 3500 RPM and mixed until the batch temperature reached 71°C (160°F.) (about 10 minutes).The speed of the mixer was then reduced to 500 revolutions per minute and the pigment pastes, plasticizer and stabilizer were added slowly over a period of about 5 minutes. The speed was then increased to 2000-3000 rpm and the material mixed until the batch temperature reached 127°C (260°F.) (approximately 15 minutes additional). The speed was then reduced to 500 RPM and the material was mixed until the batch temperature cooled to 21-32°C, i.e. 70-90°F. (about 30 additional minutes).

The pearls produced were essentially spherical, dry and free running; did not exceed 1.5 mm (0.06 inch) in diameter, and had a particle size distribution range of 0.1 to 1 mm (.004 to .040 inch)
The following table summarizes the process parameters employed:

| | | | |
|---|---|---|---|
| Equipment: | High intensity mixer | | |
| | 9.8 litre (2.6 gal.) volume | | |
| | 1.36Kg (3 lbs) loading | | |

| Elapsed Time Min. | Temperature | | Speed Rev/Min |
|---|---|---|---|
| | °C | °F | |
| 0 | ∼21 | ∼70 | 3500 |
| 10 | 71 | 160 | 500 pigments, plasticizer and stabilizer added |
| 15 | 127 | 260 | 2000-3000 |
| 30 | | | 500 cooling |
| 60 | ∼21 | ∼70 | - |

Examples 1 and 2 demonstrate decorative, inlaid floor coverings which constitute highly preferred embodiments of this invention and which comprise:
a) a substrate sheet of conventional type non-asbestos felt,
b) a gelled, thin, white, or tinted, printable plastisol coating over said substrate, prepared from effective amounts of a formulation comprising:
   - an emulsion type PVC,
   - a PVC extender, preferably having a k value about 60,
   - a plasticizer, preferably a phthlate such as di(2-ethylhexyl) phthlate or butyl benzyl phthalate,
   - a pigment, preferably titanium dioxide,
   - crystalline calcium carbonate, and
   - a barium-zinc type stabilizer
c) a print layer of one or more inks made from effective amounts of a formulation comprising:
   - a PVC-PVAc resin copolymer,
   - one or more pigments,
   - a solvent, preferably consisting essentially of methyl ethyl ketone and xylene, and
   - a dispersion aid;
d) a gelled adhesive layer made from effective amounts of a formulation comprising:
   - a PVC dispersion,
   - a PVC extender, preferably having a k value about 60,
   - a plasticizer, preferably butyl benzyl phthalate or di-isononyl phthalate, and
   - a barium-zinc type stabilizer, and
e) a mixture of gelled, transparent and colored pearls, wherein the pearls are about 50% transparent and about 50% colored, evenly distributed on the adhesive layer, prepared from effective amounts of a formulation comprising:
   - a PVC suspension resin, preferably coarse and having a k value about 65,
   - a plasticizer, preferably butyl benzyl phthalate,
   - a barium-zinc stabilizer, and, optionally,
   - a pigment or a color selected from the group consisting of red iron oxide, yellow iron oxide, chrome yellow, molybdate orange, carbon black, titanium oxide, quinanthrone red, phthallo blue and phthallo green.

Although the forgoing discussion describes this invention in terms of floor or wall covering products, this invention is intended to encompass any covering including, but not necessarily limited to, floor or wall covering, which incorporates a matrix layer of discrete, low aspect ratio resinous particles embedded in a resinous coating.

## Claims

1. A decorative, inlaid floor or wall covering which comprises:
a) a substrate
b) a printed layer in the form of a pattern applied over said substrate, and
c) an adhesive matrix layer overlaying said printed layer, in which are embedded resinous particles generally having an aspect ratio no greater than 2:1,
wherein the adhesive matrix layer extends over the whole area of the decorative covering, the embedded resinous particles are distributed over the whole area of the decorative covering, the underprint is visible through said adhesive matrix layer.

2. A decorative, inlaid floor or wall covering which comprises:
a) a substrate
b) a printed layer in the form of a pattern applied over said substrate, and
at least one layer above said printed layer, comprising
c) an adhesive matrix layer overlaying said printed layer, in which are embedded resinous particles generally having an aspect ratio no greater than 2:1,
wherein the underprint is visible through said adhesive matrix layer, the said embedded resinous particles do not cause the decorative covering to have a textured surface.

3. The product of claim 2 wherein the adhesive matrix layer is applied only in selected areas to give a pattern.

4. The product of any one of claims 1 to 3 wherein the adhesive matrix layer is coated with at least one wearlayer.

5. The product of any one of the preceding claims wherein the said resinous particles are essentially spheroidal.

6. The product of any one of the preceding claims wherein the substrate is a flexible mat.

7. The product of any one of claims 1 to 5 wherein the substrate is a non-asbestos felt sheet.

8. The product of any one of the preceding claims wherein the printed layer is a gelled, resinous layer, the surface of which has been printed with an ink suitable for use in the manufacture of floor or wall covering products.

9. The product of any one of the preceding claims wherein the adhesive matrix layer contains a major amount of a homopolymer or copolymer of vinyl chloride.

10. The product of any one of the preceding claims wherein the resinous particles are a blend of pigmented and transparent particles.

11. The product of claim 10 wherein said particles are plasticized polyvinyl chloride particles having an aspect ratio no greater than 1.5:1.

12. The product of any one of the preceding claims wherein the resinous printed layer is a gelled, foamed or foamable layer and at least one of the inks is a suppressant ink.

13. The product of any one of the preceding claims wherein the particles are discrete, vinyl chloride, homopolymer or copolymer polymerization agglomerates, sized between 0.1 to 1mm (0.004 to 0.04 inches).

14. The product of any one of claims 1 to 5 wherein the substrate is a non-asbestos felt sheet substrate, the printed layer is a gelled, printable plastisol coating over said substrate with one or more solvent based polyvinyl chloride/polyvinyl acetate inks, applied to the surface of the plastisol layer, the adhesive matrix layer contains a homopolymer or a copolymer of vinyl chloride, in which are embedded the resinous particles, and wherein said particles are essentially spheroidal polyvinyl chloride homopolymer or copolymer polymerization agglomerates, sized between 0.1-1mm (0.004-0.040 inches) and the product of comprising a fused, transparent, plastisol wearlayer as a top coat.

15. The product of claim 14 wherein the ink is made from a formulation comprising:
a) a polyvinyl chloride/polyvinyl acetate copolymer resin,
b) one or more pigments,
c) one or more solvents, and
d) a dispersion aid.

16. The product of claim 15 wherein said formulation additionally comprises benzotriazole and wherein the plastisol is foamable.

17. The product of claim 14, claim 15 or claim 16 wherein the resinous particles are a blend of pigmented and transparent particles evenly distributed within the adhesive matrix layer.

18. The product of any one of claims 14 to 17 wherein the printable plastisol coating is a foamable plastisol, pregelled in a hot air oven at the surface of which is then printed using at least one solvent based polyvinyl chloride/polyvinyl acetate ink containing a chemical suppressant to locally inhibit the expansion of the foamable plastisol in preselected areas, and wherein the product is fused and foamed in a hot air oven to form an embossed pattern.

19. The product of any one of claims 1 to 7 wherein the printed layer is a foamed layer overlaying the substrate, the surface of which foamed layer is printed.

20. The product of any one of claims 14 to 19 wherein said resinous particles are plasticized polyvinyl chloride particles having an aspect ratio no greater than 1.5:1.

## Patentansprüche

1. Bodenbelag oder Wandverkleidung mit Einlege- bzw. Parkett- bzw. Mosaikdekor, umfassend:
a) ein Substrat
b) eine bedruckte Schicht in der Form eines auf dem Substrat aufgebrachten Musters und
c) eine Klebermatrixschicht über der bedruckten Schicht, in der Harzteilchen eingebettet sind, die im allgemeinen ein Längenverhältnis von nicht mehr als 2:1 aufweisen,
worin sich die Klebermatrixschicht über die gesamte Fläche des Dekorbelags bzw. der Dekorverkleidung erstreckt, die eingebetteten Harzteilchen über die gesamte Fläche des Dekorbelags bzw. der Dekorverkleidung verteilt sind und der darunterliegende Aufdruck durch die Klebermatrixschicht hindurch sichtbar ist.

2. Bodenbelag oder Wandverkleidung mit Ein lege- bzw. Parkett- bzw. Mosaikdekor, umfassend:
a) ein Substrat
b) eine bedruckte Schicht in der Form eines auf dem Substrat aufgebrachten Musters und
zumindest eine Schicht über der bedruckten Schicht, umfassend
c) eine Klebermatrixschicht über der bedruckten Schicht, in der Harzteilchen eingebettet sind, die im allgemeinen ein Längenverhältnis von nicht mehr als 2:1 aufweisen,
worin der darunterliegende Aufdruck durch die Klebermatrixschicht hindurch sichtbar ist und die eingebetteten Harzteilchen nicht bewirken, daß der Dekorbelag bzw. die Dekorverkleidung eine texturierte Oberfläche besitzt.

3. Erzeugnis nach Anspruch 2, worin die Klebermatrixschicht nur in ausgewählten Bereichen aufgebracht wird, um ein Muster zu ergeben.

4. Erzeugnis nach einem der Ansprüche 1 bis 3, worin die Klebermatrixschicht mit zumindest einer Nutz- bzw. Verschleißschicht überzogen ist.

5. Erzeugnis nach einem der vorhergehenden Ansprüche, worin die Harzteilchen im wesentlichen kugelförmig bzw. rundlich sind.

6. Erzeugnis nach einem der vorhergehenden Ansprüche, worin das Substrat eine flexible Matte ist.

7. Erzeugnis nach einem der Ansprüche 1 bis 5, worin das Substrat eine nichtasbesthältige Filzbahn ist.

8. Erzeugnis nach einem der vorhergehenden Ansprüche, worin die bedruckte Schicht eine gelierte Harzschicht ist, deren Oberfläche mit einer Farbe bedruckt wurde, die sich zur Verwendung bei der Herstellung von Bodenbelag- oder Wandverkleidungserzeugnissen eignet.

9. Erzeugnis nach einem der vorhergehenden Ansprüche, worin die Klebermatrixschicht eine Hauptmenge eines Homo- oder Copolymers von Vinylchlorid enthält.

10. Erzeugnis nach einem der vorhergehenden Ansprüche, worin die Harzteilchen ein Gemisch aus pigmentierten und transparenten Teilchen sind.

11. Erzeugnis nach Anspruch 10, worin die Teilchen plastifizierte Polyvinylchlorid-Teilchen mit einem Längenverhältnis von nicht mehr als 1,5:1 sind.

12. Erzeugnis nach einem der vorhergehenden Ansprüche, worin die bedruckte Harzschicht eine gelierte, geschäumte oder schäumbare Schicht ist und zumindest eine der Farben eine hemmstoffhältige Farbe ist.

13. Erzeugnis nach einem der vorhergehenden Ansprüche, worin die Teilchen einzelne Vinylchlorid-Homopolymer- oder -Copolymer-Polymerisationsagglomerate mit einer Größe von 0,1 bis 1 mm (0,004 bis 0,04 Zoll) sind.

14. Erzeugnis nach einem der Ansprüche 1 bis 5, worin das Substrat ein nichtasbesthältiges Filzbahnsubstrat ist, die bedruckte Schicht eine gelierte, bedruckbare Plastisolbeschichtung über dem Substrat mit einer oder mehreren Polyvinylchlorid/Polyvinylacetat-Farben auf Lösungsmittelbasis ist, die auf der Oberfläche der Plastisolschicht aufgebracht sind, die Klebermatrixschicht, in der die Harzteilchen eingebettet sind, ein Vinylchlorid-Homopolymer oder -Copolymer enthält, und worin die Teilchen im wesentlichen kugelförmige bzw. rundliche Polyvinylchlorid-Homopolymer- oder -Copolymer-Polymerisationsagglomerate mit einer Größe von 0,1 bis 1 mm (0,004 bis 0,040 Zoll) sind und das Erzeugnis eine aufgeschmolzene, transparente Plastisol-Nutz- bzw. Verschleißschicht als Deckschicht umfaßt.

15. Erzeugnis nach Anspruch 14, worin die Farbe aus einer Formulierung besteht, umfassend:
a) ein Polyvinylchlorid/Polyvinylacetat-Copolymerharz,
b) ein oder mehrere Pigmente,
c) ein oder mehrere Lösungsmittel und
d) eine Dispersionshilfe.

16. Erzeugnis nach Anspruch 15, worin die Formulierung zusätzlich Benzotriazol umfaßt und das Plastisol schäumbar ist.

17. Erzeugnis nach Anspruch 14, 15 oder 16, worin die Harzteilchen ein Gemisch aus pigmentierten und transparenten Teilchen sind, die gleichmäßig in der Klebermatrixschicht verteilt sind.

18. Erzeugnis nach einem der Ansprüche 14 bis 17, worin die bedruckbare Plastisolbeschichtung ein in einem Heißluftofen vorgeliertes, schäumbares Plastisol ist, dessen Oberfläche dann unter Verwendung zumindest einer Polyvinylchlorid/Polyvinylacetat-Farbe auf Lösungsmittelbasis bedruckt ist, die einen chemischen Hemmstoff enthält, um die Ausdehnung des schäumbaren Plastisols in vorbestimmten Bereichen lokal zu hemmen, und worin das Erzeugnis in einem Heißluftofen geschmolzen und geschäumt wird, um ein geprägtes Muster zu bilden.

19. Erzeugnis nach einem der Ansprüche 1 bis 7, worin die bedruckte Schicht eine geschäumte Schicht über dem Substrat ist, deren Oberfläche bedruckt ist.

20. Erzeugnis nach einem der Ansprüche 14 bis 19, worin die Harzteilchen plastifizierte Polyvinylchlorid-Teilchen mit einem Längenverhältnis von nicht mehr als 1,5:1 sind.

## Revendications

1. Panneau de mur ou de plancher intérieur décoratif qui comprend :
a) un substrat
b) une couche imprimée sous la forme d'un motif appliqué sur ledit substrat ; et
c) une couche de matrice adhésive couvrant ladite couche imprimée, dans laquelle sont noyées des particules résineuses ayant généralement un rapport d'aspect non supérieur à 2 : 1,
où la couche de matrice adhésive s'étend sur la surface entière du panneau décoratif, les particules résineuses noyées sont distribuées sur la surface entière du panneau décoratif, la sous-impression est visible à travers ladite matrice adhésive.

2. Panneau de paroi ou de plancher intérieur décoratif qui comprend :
a) un substrat
b) une couche imprimée sous la forme d'un motif appliqué sur ledit substrat, et
au moins une couche au-dessus de ladite couche imprimée, comprenant
c) une couche de matrice adhésive couvrant ladite couche imprimée, dans laquelle sont noyées des particules résineuses ayant généralement un rapport d'aspect non supérieur à 2 : 1,
où la sous-impression est visible à travers ladite couche de matrice adhésive, lesdites particules résineuses noyées ne font pas que le panneau décoratif a une surface texturée.

3. Produit selon la revendication 2 où la couche de matrice adhésive est appliquée seulement sur des zones sélectionnées pour donner un motif.

4. Produit selon l'une quelconque des revendications 1 à 3 où la couche de matrice adhésive est revêtue d'au moins une couche d'usure.

5. Produit selon l'une quelconque des revendications précédentes où lesdites particules résineuses sont essentiellement sphéroïdales.

6. Produit selon l'une quelconque des revendications précédentes où le substrat est un tapis flexible.

7. Produit selon l'une quelconque des revendications 1 à 5 où le substrat est une feuille de feutre non en amiante.

8. Produit selon l'une quelconque des revendications précédentes où la couche imprimée est une couche résineuse, gélifiée, dont la surface a été imprimée avec une encre appropriée pour utilisation pour la fabrication de produits de panneau de mur ou de plancher.

9. Produit selon l'une quelconque des revendications précédentes où la couche de matrice adhésive contient une quantité majoritaire d'un homopolymère ou copolymêre de chlorure de vinyle.

10. Produit selon l'une quelconque des revendications précédentes où les particules résineuses sont un mélange de particules pigmentées et transparentes.

11. Produit selon la revendication 10 où lesdites particules sont des particules de polychlorure de vinyle plastifié ayant un rapport d'aspect non supérieur à 1,5 : 1.

12. Produit selon l'une quelconque des revendications précédentes où la couche imprimée résineuse est une couche moussable ou moussée, gélifiée et au moins une des encres est une encre supprimante.

13. Produit selon l'une quelconque des revendications précédentes où les particules sont des agglomérats de polymérisation d'un homopolymère ou d'un copolymère, de chlorure de vinyle, discrètes, d'une taille entre 0,1 et 1 mm (0,004 à 0,04 pouce).

14. Produit selon l'une quelconque des revendications 1 à 5 dans lequel le substrat est un substrat de feuille de feutre non-amianté, la couche imprimée est un revêtement de plastisol imprimable, gélifié sur ledit substrat avec une ou plus encres polychlorure de vinyle, polyvinyl acétate à base de solvant, appliquées à la surface de la couche de plastisol, la couche de matrice adhésive contient un homopolymère ou un copolymère de chlorure de vinyle dans lequel sont noyées les particules résineuses, et où lesdites particules sont essentiellement des agglomérats de polymérisation d'un homopolymère ou d'un copolymère de polychlorure de vinyle essentiellement sphéroïdales d'une taille entre 0,1-1 mm (0,004-0,040 pouce) et le produit comprenant une couche d'usure en plastisol, fondu, transparent, en tant que revêtement supérieur.

15. Produit selon la revendication 14 où l'encre est faite à partir d'une formulation comprenant :
a) une résine copolymère chlorure de vinyle/polyvinyl acétate,
b) un ou plus pigments,
c) un ou plus solvants, et
d) un additif de dispersion.

16. Produit selon la revendication 15 où ladite formulation comprend additionnellement du benzotriazole et où le plastisol est moussable.

17. Produit selon la revendication 14, la revendication 15 ou la revendication 16 où les particules résineuses sont un mélange de particules pigmentées et transparentes distribuées uniformément dans la couche de matrice adhésive.

18. Produit selon l'une quelconque des revendications 14 à 17 où le revêtement de plastisol imprimable est un plastisol moussable, prégélifié dans une étuve à air chaud dont la surface est ensuite imprimée en utilisant au moins une encre polychlorure de vinyle/polyvinyl acétate à base de solvant contenant un supresseur chimique pour inhiber localement l'expansion du plastisol moussable dans des zones présélectionnées, et où le produit est fondu et moussé dans une étuve à air chaud pour former un motif embouti.

19. Produit selon l'une quelconque des revendication 1 à 7 où la couche imprimée est une couche moussée couvrant le substrat, la surface de laquelle couche moussée est imprimée.

20. Produit selon l'une quelconque des revendications 14 à 19 où lesdites particules résineuses sont des particules de polychlorure de vinyle plastifié ayant un rapport d'aspect non supérieur à 1,5 :1.
